

# UNITED STATES PATENT OFFICE.

FRANK L. SORENSEN, OF DETROIT, MICHIGAN, ASSIGNOR TO THE METAL PROTECTION LABORATORIES, OF DETROIT, MICHIGAN, A CORPORATION OF MICHIGAN.

## METHOD FOR TREATING FERROUS-METAL ARTICLES.

1,380,847.

Specification of Letters Patent. Patented June 7, 1921.

No Drawing.

Application filed July 17, 1919. Serial No. 311,575.

To all whom it may concern:

Be it known that I, FRANK L. SORENSEN, a citizen of the United States, residing at Detroit, in the county of Wayne and State 5 of Michigan, have invented a certain new and useful Improvement in Methods for Treating Ferrous-Metal Articles, of which the following is a full, clear, and exact description.

10 This invention relates to the treatment of ferrous metal to prevent oxidation and has for its object the provision of a process which shall be simple and easy of performance which shall employ only simple and 15 inexpensive substances and which shall produce a surface which will be permanent either against corrosion or mechanical abrasion even when left naked, and shall also form a good base for painting, enamel- 20 ing, or other subsequent treatment, if desired.

I have discovered that if a mixture of zinc oxid and comminuted metallic zinc be made into a paste with a solution of sodium 25 hydroxid and applied with friction to an iron or steel surface, a zinc containing corrosion-resisting coating is formed. According to the best form of my invention that I have so far discovered I take of 30 sodium hydroxid one part; zinc oxid ten parts; and comminuted metallic zinc ten parts more or less. I first dissolve the sodium hydroxid in a little water, then incorporate the zinc oxid to form a smooth 35 paste, and finally add the finely divided metallic zinc with constant stirring, adding water, if necessary, from time to time, so as to produce a kind of paste. The stiffness of the paste may vary through wide 40 limits, wherefore much latitude is possible in the amount of water employed.

The surface of the metal to be treated is cleaned in any convenient manner, as by said blasting, scrubbing, grinding or acid 45 pickling. If the acid method is used, I prefer to neutralize the acid to a considerable extent before applying the coating but mere washing with water is generally sufficient, inasmuch as a small residue of acid is not 50 detrimental. The pasty mixture is then applied to the surface of the metal in any suitable manner, as by a brush, rubbing on with a cloth, or even by spraying. As soon as it is applied it is then brushed or 55 rubbed thoroughly onto the surface. This

friction appears to be very important since its effect is to accentuate the action and improve the coating. The superfluous paste may then be removed either by rinsing or spraying with water either with or without 60 brushing, when it will be found that the article has received a smooth, adherent coating which consists largely of metallic zinc and which adheres with great tenacity to the ferrous metal article and exhibits 65 great resistance to oxidizing or corroding influences. Paint, varnish and enamel adhere well to this coating without the necessity of employing any filling or foundation coating although a filler affords a better 70 coating when paint is used.

The proportions of the ingredients may vary widely and valuable results be achieved, but the resistance to the salt spray and other corrosive conditions appears to be 75 at a maximum when the proportion of caustic forms about ten per cent. of the dry mixture, although good results are obtained when the proportion varies between five and fifty per cent. I have found that other 80 zinc compounds such as the carbonate, or hydroxid can be substituted for zinc oxid and a beneficial coating obtained which is sufficient for many purposes although I do not consider the result as good as that obtained with zinc oxid. The degree of comminution may vary widely, though I prefer a rather coarse powder rather than a fine dust, inasmuch as the former gives a greater friction, but either can be used. 85

Certain other metals than zinc can be used, for example, finely divided tin, lead or antimony, in connection with their oxids, and a base of caustic soda as before, and in each case there is a similar but thinner coating obtained of the metal used having some protective value, but, of course, not possessing the peculiar protective quality which zinc exhibits in connection with ferrous metal. I have also used finely divided tin, 100 lead, and antimony with caustic soda base but without their oxids and in each case I have obtained a very thin metallic coating with a surface appearance characteristic of the metal used. Wherefore, I claim all 105 these mixtures and coatings and include all these ingredients within my general idea of process but prefer for protective purposes on ferrous metal to employ the zinc mixture. It will be noted that all the above 110

metals exhibit the property of producing a soluble compound in conjunction with the alkali used, and also of combining with the metallic compound in the presence of alkali 5 to produce an insoluble basic compound.

The alkali, metallic oxid, and water can be mixed up in advance and kept indefinitely so long as the finely divided metal is not added, but the latter should be incorporated with the mixture immediately before using, since the whole will otherwise upon exposure set into a hard mass.

It will be understood that I do not confine myself to this method of mixing since 15 the order of adding the ingredients is unimportant excepting from a standpoint of convenience, and that other changes can be made within the scope of my invention.

Having thus described my invention, what 20 I claim is:—

1. The method of providing ferrous metal articles with a corrosion resisting coating which consists in the frictional application to the surfaces of the same, of a mixture of 25 caustic alkali and water together with a second metal in finely divided form and an oxygen compound of said second metal, said second metal being of a nature which will combine with caustic alkali to produce a 30 soluble compound.

2. The method of providing ferrous metal articles with a corrosion resisting coating which consists in the frictional application to the surfaces of such articles, of a mixture 35 of caustic alkali and water together with a compound of a second metal and a finely comminuted metal of such nature as to tend to combine with such compound in the presence of alkali with the production of an in- 40 soluble compound.

3. The method of providing ferrous metal articles with a corrosion resisting coating which consists in applying thereto a mixture containing caustic alkali, water, a second 45 metal adapted to combine with such caustic alkali and an insoluble compound of some metal which is adapted to combine with caustic alkali to produce a soluble compound; second, forcing such mixture into 50 close contact with all parts of the ferrous surface; and, third, rinsing away the excessive mixture.

4. The method of providing ferrous metal articles with a corrosion resisting coating 55 which contains the step of applying thereto

frictionally a mixture of an insoluble compound of zinc with caustic alkali, water and a finely comminuted metal adapted to combine with caustic alkali.

5. The method of providing ferrous metal 60 articles with a corrosion resisting coating which consists in the frictional application to the surface thereof of a mixture of zinc oxid, caustic alkali, water and finely divided zinc.

6. The method of providing ferrous metal articles with a corrosion resisting coating which consists in the frictional application to the surface thereof of a zinc compound mixed with caustic alkali, water and finely divided zinc, the amount of the zinc compound and of metallic zinc being each from about two to about twelve times as great as 70 that of the alkali.

7. The method of providing ferrous metal 75 with a corrosion resisting coating which consists in the frictional application to the roughened surface thereof of a mixture of another metal in finely divided form together with the oxid of said other metal and caustic alkali and water, said second metal being of a nature to combine with the oxid in the presence of alkali and water with the production of an insoluble basic compound.

8. The method of providing ferrous metal 80 with a corrosion resisting coating which consists in the frictional application to the roughened surface thereof of a mixture of another metal in finely divided form together with a non-ferrous, metallic compound, caustic alkali and water, said other metal being of a nature to combine with said metallic compound in the presence of alkali and water with the production of an in- 85 soluble compound.

9. The method of providing metal with a 90 corrosion resisting coating which consists in the frictional application thereto of a mixture of another metal in finely divided form together with a compound of said other metal and caustic alkali and water.

10. The method of providing ferrous metal articles with a corrosion resisting coating which contains the step of applying thereto with friction a mixture of a zinc 105 oxygen compound, caustic alkali, water and finely divided metallic zinc.

In testimony whereof, I hereunto affix my signature.

FRANK L. SORENSEN.